

Aug. 1, 1939.

B. WENDT

2,168,182

PHOTOGRAPHIC MATERIAL FOR COLOR PHOTOGRAPHY

Filed Nov. 26, 1937

Fig. 1



Fig. 2



Bruno Wendt  
Inventor

By His Attorneys

Hutz and Joslin

## UNITED STATES PATENT OFFICE

2,168,182

PHOTOGRAPHIC MATERIAL FOR COLOR  
PHOTOGRAPHY

Bruno Wendt, Dessau, Germany, assignor, by  
mesne assignments, to Agfa Ansco Corporation,  
Binghamton, N. Y., a corporation of Delaware

Application November 26, 1937, Serial No. 176,609  
In Germany December 9, 1936

6 Claims. (Cl. 95—2)

This invention relates to color photography.

For producing subtractive multi-color photographic pictures several silver halide emulsion layers containing dyestuff components have been

5 superimposed on each other on a carrier, in particular arrangement of five super-imposed layers, namely three emulsion layers having two intermediate layers serving as filters or separating layers, has been found advantageous. It  
10 has also been proposed to arrange several sensitive silver halide emulsions in the form of small particles on a carrier. This latter photographic material has in particular the disadvantage that the pictures produced thereon show a grainy  
15 appearance.

It is an object of the present invention to provide an improved photographic material in which the disadvantages incurred with the aforementioned materials are avoided.

20 A further object is a photographic material in which the number of necessary emulsion layers is decreased in comparison with the hitherto used multi-layer materials.

A further object is to provide a material in  
25 which the grainy structure of one layer is made to disappear substantially.

Further objects reside in the preferred and suitable arrangement of the layers in the photographic element.

30 Further objects will be apparent from the detailed specification following hereafter.

The invention consists in arranging several sensitive silver halide emulsions having dyestuff components on a carrier, at least one silver  
35 halide emulsion being in the form of finely subdivided particles and at least one silver halide emulsion being in the form of a layer. Thus, two differently sensitized silver halide emulsions having different dyestuff components are distributed  
40 in the form of small particles in a gelatin layer and over this one or several different sensitive emulsions having components are applied in the form of layers.

The invention will be better understood with  
45 reference to the accompanying drawing, in which

Fig. 1 is a diagrammatical view of a multi-layer photographic material in an exaggerated scale and

Fig. 2 is a diagrammatical view of a single  
50 layer photographic material according to the invention.

In the figures like characters indicate corresponding parts.

In Fig. 1 *a* is a support, *b* represents a gelatin layer, *c* represents a yellow filter layer, *d* represents a blue sensitive silver halide emulsion layer, *e* indicates the particles of a silver halide emulsion sensitized to green and containing a dyestuff component fast to diffusion capable of being transformed into a purple dye, *f*

indicates the particles of a silver halide emulsion sensitized to red and containing a dyestuff component for blue-green of the kind herein referred to.

In Fig. 2 *a* is a support, *g* represents a blue-sensitive silver halide emulsion layer containing a dyestuff component capable of yielding a yellow dye, *h* indicates the particles of a silver halide emulsion sensitized to green and dyed yellow, said particles containing a dyestuff component 10 adapted to form a purple picture, *i* indicates the particles of a silver halide emulsion sensitized to red and dyed yellow, said particles containing a dyestuff component for the blue-green picture.

A suitable photographic material, for example, 15 comprises on a carrier a layer of a mixture of particles distributed in gelatin of a green-sensitive hardened silver halide emulsion provided with a dyestuff former fast to diffusion and capable of conversion into a purple dyestuff and 20 a red-sensitive hardened silver halide emulsion provided with a dyestuff former fast to diffusion and capable of conversion into a blue-green dyestuff, and over this a yellow-dyed layer, and above this again a layer of a blue-sensitive silver 25 halide emulsion provided with a dyestuff former capable of conversion into a yellow dyestuff. Preferably the yellow-dyed layer and the layer consisting of a blue-sensitive silver halide emulsion provided with a dyestuff former capable of 30 conversion into a yellow dyestuff are united to a single layer by dyeing this single layer yellow and providing it with a dyestuff former capable of conversion into a yellow dyestuff.

A single layer material for color photography 35 may be made by distributing emulsion particles of a pre-sensitized yellow-dyed silver halide emulsion containing a dyestuff former capable of conversion into a purple dyestuff and the particles of a red-sensitized yellow-dyed silver halide 40 emulsion containing a dyestuff former capable of conversion into a blue-green dyestuff in a blue-sensitive silver halide emulsion containing a dyestuff former capable of conversion to a yellow dyestuff. In this case it is of advantage that 45 the blue-sensitive emulsion constituent should constitute more than one-third of the total mass of emulsion.

As dyestuff formers for these silver halide emulsion layers there may be used with advantage components which by introduction of certain radicals have been made fast to diffusion as regards the binding agent. As described in U. S. patent application Ser. No. 72,718 filed April 4, 1936, there may be introduced into the dyestuff 50 components groups which lend a substantive character to the molecule of the dyestuff former. As described in U. S. patent application Ser. No. 90,726 filed July 15, 1936, the dyestuff components may be made fast to diffusion by introduc- 55

ing radicals of highly polymeric carboxylic acids or their derivatives. Further, dyestuff components are fast to diffusion when, as described in U. S. patent application Ser. No. 94,340 filed 5 August 5, 1936, they contain carbon chains of more than 5 carbon atoms or, according to U. S. patent application Ser. No. 158,860 filed August 13, 1937, polypeptide radicals or as described in U. S. patent application Ser. No. 159,518 filed 10 August 17, 1937, carbohydrate radicals, or as described in U. S. patent application Ser. No. 164,499 filed September 18, 1937, when they contain radicals of resins or, as described in U. S. patent application Ser. No. 166,832 filed October 15, 1937, when they contain sterol radicals. Moreover, dyestuff components fast to diffusion are obtained when the dye-forming groups are coupled to yield a molecule of chain form as described in the U. S. patent application Ser. No. 171,701 filed October 29, 1937. There may also be used 20 dyestuff components fast to diffusion, as described in U. S. patent application Ser. No. 10,704 filed March 12, 1935, in which case the dyestuff picture is produced by azo-coupling. In like manner there are suitable silver halide emulsions 25 which contain color formers fast to diffusion, as described in U. S. patent application Ser. No. 111,250 filed November 7, 1936, in which the color picture is produced by destroying directly or indirectly the dyestuff former or the dyestuff which has been formed over the silver image.

For example, if the three emulsions contain leuco-dyestuffs fast to diffusion which have developing properties for silver halide, there is obtained 30 a dyestuff image in the place of the silver image. The same is the case when suitable components for the color development are added to the emulsion and the development is conducted by means of a suitable developer.

40 There are obtained in this manner complementarily colored negatives from which copies may be produced on the same material which are positives in the correct colors. By destroying the colors first formed and converting the residual 45 components into dyestuffs, there is produced a positive correctly colored picture, also by development of the negative with a non-dyeing developer together with subsequent second development, for example by the process described in U. S. patent 50 applications Ser. No. 100,319 filed September 11, 1936, and Ser. No. 148,731 filed June 17, 1937.

The material is also suitable for any other process, provided a color former suitable for the process used is incorporated with the emulsion, 55 for example if, as described in the German Patent No. 396,485, there is used a color former which loses its capacity for forming the color at the places which contain silver, the residue of the dyestuff former is converted into a positive of 60 correct color. If, on the other hand, after the normal development and fixing a color former is converted into dyestuff, the dyestuff at the places occupied by the silver image may be destroyed by the same bleaching process.

65 Color formers which have a tendency to form precipitates in the gelatin may be held in solution by the usual dispersing agents, for example as described in U. S. patent application Ser. No. 72,714 filed April 4, 1936. Color formers which do 70 not possess sufficient fastness to diffusion may be made sufficiently insoluble by addition of a known precipitating agent.

The photographic material herein prescribed is applicable in all cases in which hitherto subtrac-

tive multi-color pictures have been produced directly or by means of any component color pictures or other multi-color copies.

What I claim is:

1. A light-sensitive element for color photography comprising a support and a plurality of differently sensitized emulsions containing dyestuff components fast to diffusion and capable of forming dyes selected from the group consisting of quinoneimine and azomethine dyes with the oxidation products of a developer, at least one of said silver halide emulsions being applied in the form of a layer and at least one other of said emulsions being applied in the form of finely distributed hardened particles. 15

2. A light-sensitive element for color photography comprising a support, a gelatin layer in direct contact with said support containing hardened microscopic particles of two differently sensitized silver halide emulsions, each of said 20 emulsions containing a dyestuff component fast to diffusion and capable of forming a dye selected from the group consisting of quinoneimine- and azomethine dyes with the oxidation product of a developer and at least one light-sensitive silver 25 halide emulsion layer containing a dyestuff component of the same kind.

3. A light-sensitive element for color photography comprising a support, a gelatin layer in direct contact with said support containing hardened microscopic particles of two differently sensitized silver halide emulsions, one type of particles being sensitized to green and containing a dyestuff component fast to diffusion capable of forming a purple dye and the second type being sensitized to red and containing a dyestuff component fast to diffusion capable of forming a blue-green dye, a silver halide emulsion layer on said gelatin layer containing a dyestuff component fast to diffusion and capable of forming a 40 yellow dyestuff.

4. A light-sensitive element for color photography comprising a support, a gelatin layer in direct contact with said support containing hardened microscopic particles of two differently sensitized silver halide emulsions, one type of particles being sensitized to green and containing a dyestuff component fast to diffusion capable of forming a purple dye and the second type being sensitized to red and containing a dyestuff 50 component fast to diffusion capable of forming a blue-green dye, a yellow filter layer on said gelatin layer, a silver halide emulsion layer containing a dyestuff component fast to diffusion capable of forming a yellow dyestuff. 55

5. A light-sensitive silver halide emulsion layer comprising a support, a blue-sensitive silver halide emulsion layer containing a dyestuff component fast to diffusion and capable of forming a yellow dye, microscopic particles of a hardened 60 silver halide emulsion sensitized to green and dyed yellow distributed in said emulsion layer, said particles containing a dyestuff component fast to diffusion and adapted to form a purple dye, microscopic particles of a hardened light-sensitive silver halide emulsion dyed yellow distributed in said emulsion layer, said particles containing a dyestuff component fast to diffusion and adapted to form a blue-green dye. 65

6. A light-sensitive element for color photography according to claim 5, the blue-sensitive emulsion layer comprising more than one-third 70 of the entire weight of the emulsion.

BRUNO WENDT.